

## UNITED STATES PATENT OFFICE

PAUL H. GEIGER, OF ANN ARBOR, MICHIGAN, ASSIGNOR TO THE UNION SWITCH & SIGNAL COMPANY, OF SWISSVALE, PENNSYLVANIA, A CORPORATION OF PENNSYLVANIA

## MANUFACTURE OF COPPER OXIDE RECTIFIERS

No Drawing.

Application filed October 9, 1929. Serial No. 398,576.

My invention relates to the manufacture of copper oxide rectifiers of the kind disclosed and claimed in Letters Patent of the United States No. 1,640,335, granted to L. O. Grondahl on August 23, 1927. One feature of my invention is the provision of a step in the manufacture of such rectifiers whereby an electrical characteristic of the finished rectifier may be changed.

19 I will describe certain processes embodying my invention, and will then point out the novel features thereof in claims.

In the practice of my invention, the copper blanks are first cleaned in the usual manner, preferably by dipping in an acid solution. The blanks are then treated with a salt, such, for example, as common table salt (sodium chloride having one per cent magnesium carbonate). This step may be performed, for example, by dipping the blanks in a solution made by dissolving approximately  $2\frac{1}{2}$  ounces of table salt in two gallons of water. The blanks are then dried, preferably by an air blast, whereupon they are treated in the usual manner to produce cuprous oxide thereon.

The salt may be applied by other methods. For example, it may be introduced into the furnace in which the blanks are given the usual heat treatment, or it may be spread on the blanks just before the blanks are oxidized, or it may be applied to the copper blanks by pressing the blanks against an absorbent material soaked with the salt solution.

35 The result of a large number of tests of the sodium chloride treatment shows a substantial increase in rectification ratio, this being accomplished by a decrease in the electrical resistance in both directions, the decrease being greater in the low resistance than in the high resistance direction.

40 As another example, the cleaned blanks may be dipped in a water solution of potassium iodide, one effect of which is to increase the electrical resistance of the finished rectifier.

45 In its broader aspect, my invention consists in treating a rectifier blank with a water solution of a "salt", the term salt when used

in this sense being taken to mean any chemical compound consisting of an acid radical united with one or more atoms of metals.

Having thus described my invention, what I claim is:

55 1. The method of preparing copper blanks for the manufacture of copper oxide rectifiers which consists in dipping the blanks in a solution made by dissolving approximately two and one-half ounces of table salt in approximately two gallons of water.

60 2. The method of preparing copper blanks for the manufacture of copper oxide rectifiers which consists in dipping the blanks in a sodium chloride solution.

65 3. The method of preparing copper blanks for the manufacture of copper oxide rectifiers which consists in treating the blanks with sodium chloride.

70 In testimony whereof I affix my signature.

PAUL H. GEIGER.

55

60

65

70

75

80

85

90

95

100